

# UNITED STATES PATENT OFFICE.

HUGH RODMAN, OF EDGEWOOD, PENNSYLVANIA, ASSIGNOR TO RODMAN CHEMICAL COMPANY, OF EAST PITTSBURGH, PENNSYLVANIA, A CORPORATION OF PENNSYLVANIA.

## PROCESS OF MANUFACTURING CARBURIZING MATERIAL AND OIL DISTILLATES.

1,209,336.

Specification of Letters Patent. Patented Dec. 19, 1916.

No Drawing.

Application filed May 24, 1915. Serial No. 30,039.

*To all whom it may concern:*

- Be it known that I, HUGH RODMAN, a citizen of the United States, and a resident of Edgewood, in the county of Allegheny and 5 State of Pennsylvania, have made a new and useful Invention in Processes of Manufacturing Carburizing Material and Oil Distillates, of which the following is a specification.
- 10 This invention relates to the production of petroleum products by distillation and to the simultaneous production of carburizing material, consisting of petroleum coke in which an energizing agent is incorporated.
- 15 An object of the invention is to produce a new and improved process of manufacturing carburizing material in which the material results as a by-product in the commercial distillation of oils or in which oils and other 20 hydrocarbon distillates are obtained as by-products in the manufacture of carburizing material.

Materials to be effective as carburizing compounds must contain carbon or carbonaceous substances in connection with substances or materials which render them active as carburizing agents and which for want of a better term may be termed energizing agents. It is well known that carbon, 25 in the form of coal or coke, is rendered effective as a carburizing agent when it is intimately mixed with an energizing agent, such, for example, as lime, soda ash, or barium carbonate. The coke residue resulting 30 from the destructive distillation of oil produces an excellent carburizing material 35 when intimately mixed with an energizing agent, such as above noted.

In carrying out my invention I mix a powdered or finely divided energizing agent with the petroleum base prior to the final process of distillation. The distillates liberated 40 during the operation of distilling are collected and conserved, and the final residue 45 resulting from complete or destructive distillation of the petroleum base consists of petroleum coke thoroughly impregnated with the energizing agent, or petroleum coke in which the energizing agent is 50 thoroughly incorporated.

In the commercial processes ordinarily employed for the distillation of oil the low volatile hydrocarbons are distilled off and

the oil is finally delivered to a coking still, ordinarily worked under high pressure, in 55 which the distillation is completed and in which the coke residue is obtained.

I have discovered that an effective method of making carburizing material or energized coked material is to mix a powdered or 60 finely divided energizing agent with the fluid petroleum or petroleum base prior to its destructive distillation in the coking still used in the ordinary commercial processes of oil 65 distillation. By so doing the energizing material employed will be thoroughly mixed with the distilling fluid and eventually remains in an evenly divided and uniformly extended condition throughout the mass of coke after the distilled oils have been driven 70 off. The energizing material may, of course, be put into and mixed with the fluid oil in a special apparatus, or it may be put directly into the fluid after the fluid has reached the coking still, as agitation of the fluid during 75 the boiling and distilling will effectively mix the energizer with the fluid.

One of the principal advantages of the invention is that advantage may be taken of the commercial manufacture of petroleum 80 products for the production of carburizing material, which is done very simply by mixing the energizing material with the fluid material to be distilled and allowing the two 85 materials to remain together during the agitation caused by the heating of the still and eventually to remain as a petroleum coke carrying predetermined amounts of energizing material evenly distributed throughout its mass.

My invention not only insures the production of an excellent carburizing material due to the use of this comparatively pure form of carbon, but also tends to give an unusually 90 thorough mixing of the materials used.

It also offers a very cheap and efficient method of making a carburizing material inasmuch as advantage is taken of existing well developed manufacturing processes without adding any appreciable cost to these 100 processes, and without detriment to the quantity or quality of the oil or distillates obtained.

I do not wish to limit this invention to the character or amount of energizing material added to the fluid or which eventually 105

remains disseminated throughout the coke which results from the complete distillation of the fluid, but I will state that a satisfactory material can be obtained by adding enough calcium hydrate and enough sodium carbonate in powdered form so that the coke will contain fifteen per cent. of calcium hydrate and ten per cent. of sodium carbonate. Another satisfactory mixture consists in adding enough barium carbonate to the fluid material so that the coke residue will contain forty per cent. of barium carbonate. It is obvious that the amount of energizing material added to the fluid before distilling must be based upon the ratio of coke produced to fluid distilled, which ratio will vary with the character of fluid treated.

What I claim is:—

1. The process of producing petroleum products and carburizing material which consists in adding to the petroleum a finely divided energizing agent, in subjecting the mixture to destructive distillation, in collecting the products driven off and removing the coked residue from the still.
2. The process of producing carburizing material and hydrocarbon distillates, which consists in mixing the petroleum base to be distilled with an energizing agent prior to destructive distillation, finally subjecting the base including the mixture to destructive distillation, in collecting the distillates resulting from the destructive distillation, and then removing the residue containing the energizing agent from the still in which

the destructive distillation has been completed.

3. The process of producing oil and carburizing material, which consists in mixing a finely divided energizing agent with a petroleum base, subjecting the petroleum to complete distillation, collecting the distillates, and then breaking up the residue containing the energizing agent.

4. The process of producing carburizing material and oil distillates, which consists in subjecting the oil to distillation, mixing the residue resulting after a partial distillation of the oil with finely divided energizing material, destructively distilling the mixture, and collecting the distillates and then removing the mixture of petroleum coke and energizing material from the still in which the destructive distillation has been carried forward.

5. The process of producing carburizing material, which consists in adding an energizing agent to the petroleum base to be distilled prior to the destructive distillation of the base, in carrying forward the commercial processes of oil distillation, and finally removing the coked residue mixed with energizing agent from the coking still.

In testimony whereof, I have hereunto subscribed my name this 22nd day of May, 1915.

HUGH RODMAN.

Witnesses:

E. W. McCALLISTER,  
C. W. McGHEE.